

Patented Feb. 10, 1925.

## UNITED STATES PATENT OFFICE.

FRANK T. LAHEY, OF AKRON, OHIO.

## SHEET COMPOSITION.

No Drawing.

Application filed March 29, 1923. Serial No. 328,512.

*To all whom it may concern:*

Be it known that I, FRANK T. LAHEY, a citizen of the United States of America, residing at Akron, in the county of Summit and State of Ohio, have invented certain new and useful Improvements in Sheet Compositions, of which the following is a specification.

This invention relates to a sheet composition, and the process of manufacturing the same.

More particularly, the invention has relation to a process for the utilization of waste material, such as waste unvulcanized or uncured rubber fabric.

One important object of the invention is to provide an improved process for manufacturing a sheet material from waste products combined in a novel manner.

A second important object of the invention is the production of an improved sheet material made from waste material, the principal materials being waste paper and waste rubber.

In carrying out the objects of this invention, the preferred manner of producing the sheet material, is as follows.

Sufficient of the waste material is fixed in the following proportions, and in the following way:

To each four ounces of paper board, or paper pulp and waste paper, there is added four ounces of rubber or rubber fabric of the kind known as uncured friction, or rubber fabric which consists of rubber with a fabric or fiber incorporated therein, or a mixture of four ounces of rubber with fiber may be utilized. The batch consisting of these ingredients is then placed upon a washing machine, either of the type provided with corrugated rolls, or of the type provided with smooth rolls moving at different speeds, and is passed through these rolls so as to thoroughly and intimately knead the ingredients together, and the materials being slightly moistened with water, or preferably an emulsion of various kinds of oils, either vegetable, animal or mineral. After this batch is intimately mixed and then dried, there is added to this treated rubber waste in the proportion of four ounces to each eight ounces of the mixture, this rubber waste being treated in the manner described in my prior Patent 1,233,252, of July 10, 1917. The entire batch is then placed in a mixing material, and vari-

ous oxides added thereto, or these oxides may be replaced by suitable mineral substances, these substances acting as fillers. As the examples of such substances, there may be used fossil flour, magnesia, magnesite, fuller's earth, zinc oxide, or other similar substances. Sulphur is also added according to the degree of hardness required in the resultant product. After the mixing, the material is then rolled to proper sheet form and vulcanized to the required degree of hardness, this depending of course on the sulphur content.

As an alternative manner of preparing such sheets, I may mix together two pounds of crude rubber, from two to four ounces of oleaginous substance, either in solid or liquid condition, these ingredients being heated sufficiently to liquefy the solids. To the batch thus formed, I add from four to six pounds of paper pulp in a damp condition, preferably using paper pulp which has been pulped on a washing machine by the aid of water. As an alternative to the paper pulp, I may add raw vegetable substances containing cellulose. These substances are thoroughly mixed in a mixing machine, and may also have suitable fillers, and a required quantity of sulphur for hardening purposes added thereto. The subsequent treatment after consists in rolling into sheets and vulcanizing as desired.

The resultant product from either of these alternatives may be manufactured into a variety of articles, such as roofing sheets or tiles, in which case the material is left more or less soft and pliable, into boxes in which case the vulcanization is carried to a point where the articles are hard and resistant, and in fact into a wide variety of products.

There has thus been provided a novel and improved product, and a novel process of manufacturing the same.

I claim:

1. The process of manufacturing a composition which consists in intimately mixing equal parts of paper pulp and uncured waste rubber fabric in combination with a moistening material, adding to the mixed batch a quantity of treated rubber waste equal to one-half the quantity of the batch and thoroughly mixing the entire mass together with an inert mineral filler to which has been added sulphur in desired quantities for vulcanizing, rolling the mass into

sheets, and finally vulcanizing the rolled sheets.

2. The process of preparing a composition of the class described which consists in 5 mixing equal quantities of waste from paper manufacture and uncured rubber fabric together with an oil emulsion, drying the mass, adding to the dried mass a quantity

of treated rubber waste equal in quantity to the uncured rubber fabric, mixing the 10 entire batch intimately with the addition of sulphur to a quantity sufficient to produce desired vulcanization, rolling the mixture into sheets, and vulcanizing the sheets.

In testimony whereof I affix my signature.  
FRANK T. LAHEY.